

**[54] REFRIGERATION OIL COMPOSITION  
HAVING WIDE BOILING RANGE**

[75] Inventors: **Ivor W. Mills; John J. Melchiore**,  
Marcus Hook, Pa.

[73] Assignee: **Sun Oil Company**, Philadelphia, Pa.

[22] Filed: **Aug. 12, 1970**

[21] Appl. No.: **63,303**

[52] U.S. Cl. .... **208/14**, 208/19, 252/68

[51] Int. Cl. .... **C10g 41/00**

[58] Field of Search .... **252/67; 208/14, 19, 15**

**[56] References Cited****UNITED STATES PATENTS**

|           |         |                 |       |        |
|-----------|---------|-----------------|-------|--------|
| 3,224,955 | 12/1965 | Anderson        | ..... | 208/28 |
| 3,196,102 | 7/1965  | Mills et al.    | ..... | 208/14 |
| 3,145,161 | 8/1964  | Anderson et al. | ..... | 208/14 |

*Primary Examiner*—Herbert Levine

*Attorney*—George L. Church, Donald R. Johnson,  
Wilmer E. McCorquodale, Jr. and Barry A. Bisson

**[57] ABSTRACT**

A wide boiling range e.g., for a given VGC) refrigeration oil, having good chemical and thermal stability and good miscibility with fluorinated hydrocarbon refrigerants, comprises a blend of from 50–75 volume percent of hydrorefined naphthenic oil component and 50–25 volume percent of solvent refined and dewaxed paraffinic oil component. Preferably, the hydrorefined naphthenic oil component (which can be a blend of two or more hydrorefined oils) has an SUS viscosity at 100° F. in the range of 75–750 SUS and the paraffinic oil component (which can be a blend) is chosen so that the resulting naphthenic paraffinic blend has a viscosity at 100° F. in the range of 100–500 SUS (preferably 125–300 SUS, typically 150–250 SUS) and has a maximum natural floc point of –35° F. Preferably the blend contains less than 10 ppm (more preferably less than 5) of basic nitrogen and contains in the range of 15–35 weight percent aromatics.

**9 Claims, No Drawings**

REFRIGERATION OIL COMPOSITION HAVING  
WIDE BOILING RANGECROSS REFERENCE TO RELATED  
APPLICATIONS

The following patents and applications, all assigned to The Sun Oil Company (as is the present application), are related to the disclosure of the present application in that they disclose methods of obtaining hydrorefined naphthenic oils, dewaxed paraffinic oils and methods of reducing the basic nitrogen content of component oils which can be used to make the blended refrigeration oil composition of the present invention. Other methods for obtaining hydrorefined naphthenic and dewaxed paraffinic oils, useful as such blending components, are well known to the art.

The disclosure of all of the following applications and patents is hereby incorporated in the present application:

| Serial No. | Filing Date | Patent No. | Issue Date | Title/Inventor (s)                                                                                                                                        | 10 | 20     | 30      | 40                                       | 50 | 60 |
|------------|-------------|------------|------------|-----------------------------------------------------------------------------------------------------------------------------------------------------------|----|--------|---------|------------------------------------------|----|----|
| 622,398    | 3-13-67     | 3,462,358  | 8-19-69    | Clay Treatment of Hydro-refined Cable Oils - IVOR W. MILLS & GLENN R. DIMELER                                                                             | 25 | 22,295 | 3-24-70 | BACKGROUNDS AND SUMMARY OF THE INVENTION |    |    |
| 636,493    | 5-5-67      |            |            | Process for Preparing an Aromatic Oil and Non-discoloring Rubber Composition Containing Said Oil - IVOR W. MILLS, GLENN R. DIMELER & MERRITT C. KIRK, JR. | 30 | 35,231 | 5-6-70  |                                          |    |    |
| 652,026    | 7-10-67     | 3,502,567  | 3-24-70    | Process for Producing Cable Oils by Sequential Refining Steps - IVOR W. MILLS & GLENN R. DIMELER                                                          | 35 |        |         |                                          |    |    |
| 657,438    | 5-29-67     |            |            | Rubber Containing Acid-Treated Oils and Its Preparation - ABRAHAM SCHNEIDER & ARCHIBALD P. STUART                                                         | 40 |        |         |                                          |    |    |
| 730,999    | 5-22-68     |            |            | Hydrorefined Transformer Oil and Process of Manufacture - IVOR W. MILLS & GLENN R. DIMELER                                                                | 45 |        |         |                                          |    |    |
| 812,516    | 2-19-69     |            |            | Catalytic Hydrofinishing of Petroleum Distillates in the Lubricating Oil Boiling Range - IVOR W. MILLS, MERRITT C. KIRK, JR. & ALBERT T. OLENZAK          | 50 |        |         |                                          |    |    |
| 828,746    | 5-28-69     |            |            | Isomerization of Waxy Lube Streams and Waxes - IB STEINMETZ & DAVID S. BARMBY                                                                             | 55 |        |         |                                          |    |    |
| 850,716    | 8-18-69     |            |            | Blended Hydrocarbon Oil and Process of Manufacture - IVOR W. MILLS & GLENN R. DIMELER                                                                     | 60 |        |         |                                          |    |    |
|            |             |            |            |                                                                                                                                                           | 65 |        |         |                                          |    |    |

The present invention relates to a refrigeration oil which has good chemical stability and also good thermal stability and which has a wider boiling range for a given VGC than does a prior art "paraffinic" refrigeration oil. The novel oil also retains a floc point no

Hydrorefined Lube Oil and Process of Manufacture - IVOR W. MILLS & GLENN R. DIMELER

Process for Preparing High Viscosity Hydrorefined Cable Oil - IVOR W. MILLS, GLENN R. DIMELER, WILLIAM A. ATKINSON & DAVID A. HOFFMAN

Oil and Process of Manufacture of Blended Hydro-refined Oil - IVOR W. MILLS & GLENN R. DIMELER

Light-colored Highly Aromatic Oil and Process of Preparation - IVOR W. MILLS, GLENN R. DIMELER & MERRITT C. KIRK, JR.

Hydrorefined Cable Oil and Process of Manufacture - IVOR W. MILLS & GLENN R. DIMELER

Hydraulic Oil Composition Containing a Blended Base Stock - JOHN Q. GRIFFITH, III, EDWARD S. WILLIAMS, WILLIAM H. REILAND, JR., IVOR W. MILLS & GLENN R. DIMELER

greater than  $-35^{\circ}$  F. (more preferred less than  $-40^{\circ}$  F.), has good miscibility with conventional refrigerants, has good sealed tube stability and permits the operation of compressors at higher operating temperatures (e.g. a coil temperature above  $125^{\circ}$  C.) than do present refrigeration oils.

A wide boiling range (e.g. for a given VGC) refrigeration oil of the present invention, having good chemical and thermal stability and good miscibility with fluorinated hydrocarbon refrigerants, comprises a blend of from 50-75 volume percent of hydrorefined naphthenic oil component and 50-25 volume percent of a dewaxed paraffinic oil component. Preferably, the hydrorefined naphthenic oil component (which can be a blend of two or more hydrorefined oils) has an SUS viscosity at  $100^{\circ}$  F. in the range of 75-750 SUS and the paraffinic oil component is chosen so that the resulting naphthenic-paraffinic blend has a viscosity at  $100^{\circ}$  F. in the range of 100-500 SUS (preferably 125-300 SUS, typically 150-250 SUS) and has a maximum natural (e.g. does not contain a pour point depressant) floc point of  $-35^{\circ}$  F. Preferably the blend contains less than 10 ppm (more preferably less than 5) of basic nitrogen and contains in the range of 15-35 weight percent aromatics. The paraffinic oil component can contain or consist of hydrorefined paraffinic oil having a low wax content. The hydrorefined naphthenic component can be a raffinate from solvent extraction (either before or after hydrorefining), as with furfural, to reduce the aromatic content.

The novel oil can be made by blending a low basic nitrogen content paraffinic oil (having a viscosity at  $100^{\circ}$  F. of about 500 SUS) with a low basic nitrogen content hydrorefined naphthenic oil (e.g. having an SUS viscosity at  $100^{\circ}$  F. of about 150). A preferred process for insuring a low basic nitrogen content (e.g. less than 5 ppm, typically 1 ppm or less) in the naphthenic and paraffinic components and/or in the blend comprises acid or acid-clay contacting the blend and/or one or more of the component oils. For example, the Lewis acid contacting (preferably with neutralization) of the aforementioned applications Serial Nos. 622,398 (now U.S. Pat. No. 3,462,358); 652,026 (now U.S. Pat. No. 3,502,567); 657,438; 850,717 and 850,779. A preferred method of reducing the basic nitrogen in a blend of a hydrorefined naphthenic oil and a dewaxed paraffinic oil or in one or both of these component oils is to contact the oil with an adsorbent comprising an acid-activated adsorbent clay, more preferably an admixture or combination of an acid-activated adsorbent clay and a fuller's earth bleaching clay such as attapulgite. Useful adsorbent admixtures and process conditions for such contacting are disclosed in U.S. Pat. No. 3,369,999, for the decolorizing of waxes.

#### FURTHER DESCRIPTION

One important test of refrigeration oil quality is the floc point, which is a measure of the tendency of wax separation from the oil under conditions which simulate actual operation in a refrigeration system. A second important test, which can be correlated with actual use conditions, is the 14-day sealed tube stability test.

The floc point is the temperature at which a floc of wax or other solid substances separates from a 10 percent mixture of the oil in R-12 refrigerant ( $CCl_2F_2$ ). Lint-like floc is to be contrasted with cloud-like haze. The test apparatus comprises a 15 ml graduated tube, 27.9 cm  $\times$  14 mm with 2 mm thick walls, a pressure tube holder, a cooling bath, a thermometer, and a cooling coil. The cooling bath can be large, wide mouth Dewar flask (Fisher Scientific Co. No. 14-197, Size 2, is satisfactory). Dry ice and acetone are used as the cooling medium. The thermometer can be ASTM Low Cloud and Pour 6F, having the range  $-112^{\circ}$  to  $+70^{\circ}$  F. The R-12 cooling coil is made of one-fourth inch copper tubing, and is immersed in the dry ice acetone bath to chill the refrigerant to below  $-25^{\circ}$  F. so that it may be charged as liquid to the graduated tube containing the sample. In this test, a sample of the oil to be tested is charged to a graduated glass tube and chilled refrigerant is added. The tube is sealed in the tube holder and the system is allowed to warm enough to become homogeneous on shaking. The mixture is then cooled in a chilling bath until there is a distinct floc present in it. The temperature at that point is reported as the floc point. Since considerable pressure is developed in the glass tube during the test, the tube should be wrapped with a cloth towel when it is removed from the cooling bath. The operator should wear a protective face mask.

The procedure involves pipeting 1 cc of the oil to be tested to the glass tube. The glass tube and sample are inserted into the pressure tube holder and the assembly is immersed into the cooling bath and chilled to a temperature below the boiling point of the refrigerant ( $-25^{\circ}$  F for R-12). The refrigerant is condensed by passing it slowly through the copper cooling coil and the liquid is added to the cooled sample tube until the liquid level reaches the 10 cc mark on the tube. That is, total volume of the oil-refrigerant mixture is 10 cc. The charged tube is then tightly sealed and allowed to warm up to a temperature sufficiently high to permit making the system homogeneous by shaking. The assembly with the refrigerant-sample mixture is then cooled in the dry ice-acetone bath. The temperature of the bath is lowered at a rate of approximately 1 or  $2^{\circ}$  Fahrenheit per minute by careful addition of dry ice. Observations are made at  $1^{\circ}$  intervals, beginning at  $0^{\circ}$  F. When such observations first reveal a distinct flocculent material suspended in the mixture, the reading of the test thermometer in the bath is recorded as the floc point. This floc point test is reproducible within at least  $2^{\circ}$  F. Some oils show a haze at a temperature slightly above the floc point temperature. This temperature is usually 5 to 10 above the actual floc point. If a test oil clouds at about  $0^{\circ}$  F, the test should be repeated to be certain that moisture has not been inadvertently introduced into the test apparatus.

The second important test, the 14-day sealed tube stability, rates the quality of a refrigeration oil by evaluation of the appearance of the oil and a metal test strip, and the amount of reaction of an oil with a halogenated refrigerant after aging in a sealed tube.

Since oil and gases are under pressure in the glass tubes, the tubes should be treated as though they might explode at any time. Safety glasses, a plastic face shield and heavy leather gloves should be worn when handling a sealed tube.

The method consists of sealing 5 ml of an oil, "R-12" refrigerant, and a steel strip in a heavy-walled glass tube which is then heated in an oven to  $347^{\circ} + 1^{\circ}$  F. and aged at the temperature for 14 days. The oil is rated on appearance at 14 days. After 14 days the tubes are opened and the contents analyzed by vapor phase chromatography for the percentage of R-22 and R-12, thus determining the composition of R-12 ( $\text{CCl}_2\text{F}_2$ ) to R-22 ( $\text{CHClF}_2$ ). The detailed procedure for the sealed tube stability test is well known in the refrigeration manufacturing and petroleum refining industries. For example, the procedure was reported and published in print by H. O. Spauschus and G. C. Doderer, at the 73rd ASHRAE Annual Meeting, Toronto, Ontario, June 28, 1966.

In the oil of the present invention, it is important that either the blended oil or all of its components be as free of basic nitrogen as is practical. Preferred means of reducing basic nitrogen being contacting with acid (e.g.  $\text{H}_2\text{SO}_4$ ) and neutralization, or by contacting with an acid-activated clay (preferably a mixture of acid-activated clay and attapulgite). Such contacting to reduce the basic nitrogen in the oil insures good 14 day sealed tube stability (e.g. maximum of 2.5 percent R-22, more preferably 1.5 percent maximum, typically less than 1.0 percent).

The acid or acid clay treatment of the paraffinic component also causes improved results in the Falex failure load test, which is a test to determine lubricating quality of a refrigeration oil.

#### ILLUSTRATIVE EXAMPLES

In the following examples, SUS viscosity is at  $100^{\circ}$  F. and parts are by volume, unless otherwise indicated.

#### EXAMPLE 1

A hydrorefined naphthenic oil component having a viscosity of 150 SUS was obtained by blending 100 SUS and 500 SUS hydrorefined naphthenic oils. Each of these oils was obtained by severe hydrorefining (as defined in U.S. Pat. No. 3,462,358) of naphthenic acid-free naphthenic distillate. The hydrorefining was at  $625^{\circ}$  F., 1,200 psig of 80 percent hydrogen, 0.25 LHSV, in the presence of sulfided NiMo oxide catalyst. The 150 SUS blended composition was contacted at about  $240^{\circ}$  F. with a mixture, per barrel of oil, of 10 pounds of acid-activated clay and 10 pounds of attapulgite. The resulting clay contacted 150 SUS hydrorefined naphthenic oil contained less than 1 ppm of basic nitrogen.

A Duosol solvent refined and methylethyl ketone dewaxed (to a pour point of  $0^{\circ}$  F.) paraffinic lube distillate, having a SUS viscosity of 500, was contacted at  $240^{\circ}$  F. with a mixture, per barrel of oil, of 10 pounds of acid-activated clay and 10 pounds of attapulgite. The resulting 500 SUS paraffinic component contained less than 1 ppm of basic nitrogen.

A blended refrigeration oil, of the present invention, was obtained by blending 68 parts by volume of the 150 SUS hydrorefined naphthenic oil component and 32 parts of the 500 SUS paraffinic component. The properties of this blended refrigeration oil are reported in Table 1, along with a typical range of properties of a preferred blended refrigeration oil composition.

Table 2 hereof reports the distillation ranges in °F., obtained under vacuum and corrected to at 1 at-

mosphere, of the hydrorefined naphthenic component, the refrigeration oil blend and the dewaxed paraffinic component. Note the wide boiling range of the blended refrigeration oil, compared with the boiling range of each component. In one preferred embodiment, at least 80 volume percent of the naphthenic component will distill below  $800^{\circ}$  F., corrected to 1 atmosphere, and at least 80 volume percent of the paraffinic component will distill above  $800^{\circ}$  F., corrected to one atmosphere the latter requirement being the most important. More preferred, at least 50 percent of the paraffinic component should boil above  $900^{\circ}$  F.

#### EXAMPLE 2

A blended refrigeration oil was obtained as in Example 1, except that the blend contained 63 parts of the 150 SUS hydrorefined naphthenic oil component and 37 parts of the 500 SUS dewaxed paraffinic component. This blended refrigeration oil had the same properties as those reported in Table 1 for the oil of Example 1 except that the viscosity at  $100^{\circ}$  F. was 235°, the pour point was  $-25^{\circ}$  F., the aniline point was  $199.8^{\circ}$  F. and the weight percent (gel) aromatics was 27.5.

The performance of the blended refrigeration oil of this example was evaluated after 2,000 hours of operation with R-12 in a compressor at a coil temperature of about  $160^{\circ}$  C. The condition of the Mylar, the valves, the copper plating on the shafts and of the other operating parts after the 2,000 hours was significantly better than the condition of similar parts from a compressor run for 2,000 hours at  $160^{\circ}$  C. using a conventional naphthenic refrigerant (which failed before 2,000 hours).

In another series of "use tests," the blended refrigeration oil of this example was compared with a low basic nitrogen content dewaxed paraffinic refrigeration oil and with a refrigeration oil comprising 60 percent alkylated benzene and 40 percent mineral oil. The tests were run for 3 months at  $160^{\circ}$  C. winding temperature. The naphthenic-paraffinic blend of the present invention exhibited better wear and life properties than did the other two oils.

This was a severe test of thermal stability since these compressors normally operate within the  $130^{\circ}$ – $140^{\circ}$  C. temperature range. Generally, prior art naphthenic refrigeration oils are used in compressors where the temperature is in the  $100^{\circ}$ – $110^{\circ}$  C. range.

TABLE I  
TYPICAL PROPERTIES OF BLENDED  
REFRIGERATION OIL

| Test                             | Method*    | Example 1<br>Blended<br>Refrigeration<br>Oil | Typical<br>Range |
|----------------------------------|------------|----------------------------------------------|------------------|
| Viscosity, SUS/ $100^{\circ}$ F. | D2161      | 227                                          | 210–240          |
| Viscosity, SUS/ $210^{\circ}$ F. | D2161      | 46                                           | 45–52            |
| Flash, COC, °F.                  | D92        | 355                                          | 340 min          |
| Fire, COC, °F.                   | D92        | 390                                          | —                |
| Pour, °F.                        | D97        | –35                                          | –25 max          |
| Viscosity-gravity<br>Constant    | calculated | 0.847                                        | —                |
| Color                            | D1500      | L 1.0                                        | 2.0 max          |
| Gravity, °API                    | D287       | 26.0                                         | 25–27            |
| Total Acid No.,<br>mgKOH/g       | D974       | 0.00                                         | 0.05 max         |
| Dielectric Strength,<br>KV       | D877       | 30                                           | 25 min           |
| Inorganic Chloride &             |            |                                              |                  |

|                                |       |        |         |
|--------------------------------|-------|--------|---------|
| Sulfates                       | D878  | None   |         |
| Basic Nitrogen, ppm            | **    | 1      |         |
| Free Sulfur                    | D989  | None   |         |
| Corrosive Sulfur; Class        | D1275 | No. 1  |         |
| Total Sulfur, %                | D129  | 0.04   |         |
| Aniline Point, °F.             | D611  | 195    |         |
| Refractive Index               | D1747 | 1.4945 |         |
| Aromatics, Gel. %              |       | 30     |         |
| Floc, °F.                      | **    | -47    | -35 max |
| Power Factor/25°C., Initial    | D924  | 0.001  |         |
| Power Factor/100°C., Initial   | D924  | 0.0086 |         |
| 14-Day Sealed Tube, wt. & R-22 | **    | 0.6    | 1.0 max |

\* ASTM Test Designations

\*\* Floc and sealed tube tests are with R-12 refrigerant and are described in this specification. The basic nitrogen test is described in Serial No. 850,779.

TABLE 2  
DISTILLATION RANGES FOR EXAMPLE 1  
COMPONENTS AND BLEND

°F. at 760 MM\*

| Hydrorefined Naphthenic Component | Refrigeration Oil Blend of Example 1 | Dewaxed paraffinic Component |      |
|-----------------------------------|--------------------------------------|------------------------------|------|
| Initial                           | 581                                  | 561                          | 744  |
| 5%                                | 632                                  | 606                          | 801  |
| 10                                | 650                                  | 632                          | 844  |
| 20                                | 674                                  | 667                          | 887  |
| 30                                | 690                                  | 695                          | 908  |
| 40                                | 705                                  | 726                          | 922  |
| 50                                | 721                                  | 760                          | 933  |
| 60                                | 736                                  | 808                          | 946  |
| 70                                | 755                                  | 861                          | 959  |
| 80                                | 777                                  | 908                          | 975  |
| 90                                | 803                                  | 957                          | 100  |
| 95%                               | 826                                  | 980                          | 1021 |
| Final                             | 842                                  | 993                          | 1037 |

\* The distillations were made at reduced pressure and corrected (or extrapolated) to one atmosphere.

40

The invention claimed is:

1. A composition, useful as a refrigerator oil, comprising a blend of from 50-75 volume percent of a hydrorefined naphthenic oil and from 50-25 percent of a dewaxed paraffinic oil, said blend containing in the range of 15-35 weight percent aromatics, having an SUS viscosity at 100° F. in the range of 100-500 and a natural floc point no higher than -35° F. in  $CCl_2F_2$  refrigerant.
- 5 2. The composition of claim 1 and having a basic nitrogen content no greater than 10 ppm.
3. The composition of claim 2 wherein no greater than 2.5 Wt.  $CHClF_2$  is determined after 14-days of sealed tube stability testing at 347° F. with  $CCl_2F_2$  refrigerant in the presence of a steel strip.
- 10 4. The composition of claim 1 and having better thermal stability than a naphthenic refrigeration oil of about the same viscosity at 100° F.
5. The composition of claim 4 and which, compared 20 with said naphthenic refrigeration oil, produces significantly less coke deposit on throttle valves when used for about 2,000 hours in a compressor which is operated at an average coil temperature in the range of 140°-170° F.
- 25 6. The composition of claim 5 wherein the basic nitrogen content is less than 5 ppm and wherein no greater than 1.0 Wt. percent of  $CHClF_2$  is determined after 14-days of sealed tube stability testing at 347° F. with  $CCl_2F_2$  refrigerant in the presence of a steel strip.
- 30 7. A composition according to claim 1 wherein said hydrorefined naphthenic oil has a viscosity at 100° F. in the range of 100-750 SUS and wherein at least 50 volume percent of said dewaxed paraffinic oil distills above 900° F., the distillation being corrected to one atmosphere.
- 35 8. A composition according to claim 7 and having a viscosity at 100° F. in the range of 125-300 SUS.
9. A composition according to claim 1 and having a viscosity at 100° F. in the range of 150-250 SUS.

\* \* \* \* \*